

# United States Patent

[19]

Niebyski

[11] 3,948,618

[45] Apr. 6, 1976

[54] **FUEL COMPOSITIONS CONTAINING  
GLYCERIDES FOR REDUCING THE  
PLUGGING OF EXHAUST GAS CATALYSTS**

[75] Inventor: **Leonard M. Niebyski**, Birmingham,  
Mich.

[73] Assignee: **Ethyl Corporation**, Richmond, Va.

[22] Filed: **June 5, 1975**

[21] Appl. No.: **584,140**

[52] U.S. Cl. .... **44/66; 44/68; 44/70;**  
252/386

[51] Int. Cl.<sup>2</sup> .... **C10L 1/18**

[58] Field of Search .... **44/66, 68, 70; 252/386**

[56] **References Cited**

UNITED STATES PATENTS

1,692,784 11/1928 Orelup et al. .... 44/66

|           |         |                   |       |
|-----------|---------|-------------------|-------|
| 1,995,615 | 3/1935  | Jaeger .....      | 44/70 |
| 2,527,889 | 10/1950 | Moore et al. .... | 44/66 |
| 2,747,979 | 5/1956  | Thompson .....    | 44/70 |
| 3,222,146 | 12/1965 | Case et al. ....  | 44/70 |

*Primary Examiner*—Daniel E. Wyman

*Assistant Examiner*—Y. H. Smith

*Attorney, Agent, or Firm*—Donald L. Johnson; Robert A. Linn

[57] **ABSTRACT**

Gasoline compositions containing cyclopentadienyl manganese tricarbonyl antiknock and a glyceride ester in an amount sufficient to alleviate the plugging of catalysts being used in an engine exhaust system to lower the amount of undesirable constituents in exhaust gas. The antiknock and glyceride are preferably added to the gasoline as an additive mixture.

**16 Claims, No Drawings**

**FUEL COMPOSITIONS CONTAINING  
GLYCERIDES FOR REDUCING THE PLUGGING  
OF EXHAUST GAS CATALYSTS**

**BACKGROUND OF THE INVENTION**

Cyclopentadienyl manganese compounds are excellent antiknocks in gasoline used to operate internal combustion engines. These manganese compounds have proved to be especially beneficial in solving some of the problems present when low-lead or lead-free gasolines are used with internal combustion engines. Use of such compounds as antiknocks is described in U.S. Pat. Nos. 2,818,417, 2,839,552, and 3,127,351, incorporated herein by reference. Not only are these compounds effective antiknock compounds, but it has also been found that they do not adversely affect the activity of oxidation metal catalysts used to decrease the amount of undesirable constituents in engine exhaust gas. Under some operating conditions it has been found that, although the manganese antiknocks do not lessen the activity of the exhaust gas catalyst, they can interact in some manner at the surface of the catalyst bed leading to a reduction in the size of the openings into the bed thereby causing an increase in exhaust backpressure and a decrease in the effective life of said catalysts. The present invention provides a simple effective means of alleviating this problem.

It has been previously suggested that the addition of triethyl citrate to gasoline mixes containing organomanganese antiknocks tends to reduce catalyst plugging.

**SUMMARY**

According to the present invention, the useful life of an exhaust gas catalyst in an exhaust system of an engine operating on gasoline containing a cyclopentadienyl manganese antiknock is increased by providing new additive fluids and gasoline compositions which contain a cyclopentadienyl manganese tricarbonyl and an amount of gasoline soluble glyceride ester sufficient to alleviate plugging of the exhaust gas catalyst.

**DESCRIPTION OF THE PREFERRED  
EMBODIMENTS**

The essence of the present invention resides in reducing the plugging of oxidation metal catalytic apparatus for purifying exhaust gases of internal combustion engines which burn a gasoline containing an organomanganese compound. This reduction in plugging is effected by the addition of gasoline soluble glycerides, and preferably the triglycerides, to the gasoline. Accordingly, a preferred embodiment is a gasoline suitable for use in an internal combustion engine and containing an amount of organomanganese compound, preferably a cyclopentadienyl manganese tricarbonyl, sufficient to increase its antiknock effectiveness, and also containing an amount sufficient to prevent plugging of the catalyst of gasoline soluble glycerides, preferably the triglycerides.

A further embodiment of the present invention is a gasoline additive fluid composition comprising an organomanganese compound, preferably a cyclopentadienyl manganese tricarbonyl, and most preferably methylcyclopentadienyl manganese tricarbonyl, in an amount sufficient to improve the antiknock characteristics of the gasoline and glycerides, preferably the triglycerides, and most preferably the lower glyceryl

trialkanoates such as glyceryl triacetate, in an amount sufficient to reduce catalyst plugging.

Since the invention also embodies the operation of an internal combustion engine having a catalyst unit in its exhaust system, in a manner which results in reduced plugging of the catalyst, a still further embodiment is a method of operating an internal combustion engine using a gasoline containing an antiknock amount of an organomanganese, preferably a cyclopentadienyl manganese tricarbonyl, and most preferably methylcyclopentadienyl manganese tricarbonyl antiknock in a manner which results in substantial reduction in the plugging of the catalyst, said method comprising (a) supplying to the fuel induction system of said engine a gasoline containing an organomanganese antiknock and a gasoline soluble glyceride, (b) mixing said gasoline with air, (c) inducting the mixture into the combustion chambers of said engine, (d) compressing said mixture, (e) igniting said compressed mixture, and (f) exhausting the resultant combustion products which have a reduced plugging effect on the catalyst through said catalyst.

Liquid hydrocarbon fuels of the gasoline boiling range are mixtures of hydrocarbons having a boiling range of from about 80°F. to about 430°F. Of course, these mixtures can contain individual constituents boiling above or below these figures. These hydrocarbon mixtures contain aromatic hydrocarbons, saturated hydrocarbons and olefinic hydrocarbons. The bulk of the hydrocarbon mixture is obtained by refining crude petroleum by either straight distillation or through the use of one of the many known refining processes, such as thermal cracking, catalytic cracking, catalytic hydroforming, catalytic reforming, and the like. Generally, the final gasoline is a blend of stocks obtained from several refinery processes. The final blend may also contain hydrocarbons made by other procedures such as alkylate made by the reaction of C<sub>4</sub> olefins and butanes using an acid catalyst such as sulfuric acid or hydrofluoric acid.

Preferred gasolines are those having a Research Octane Number of at least 85. A more preferred Research Octane Number is 90 or greater. It is also preferred to blend the gasoline such that it has a content of aromatic hydrocarbons ranging from 10 to about 60 volume percent, an olefinic hydrocarbon content ranging from 0 to about 30 volume percent, and a saturate hydrocarbon content ranging from about 40 to 80 volume percent, based on the whole gasoline.

In order to obtain fuels having properties required by modern automotive engines, a blending procedure is generally followed by selecting appropriate blending stocks and blending them in suitable proportions. The required octane level is most readily accomplished by employing aromatics (e.g., BTX, catalytic reformate or the like), alkylate (e.g., C<sub>6-9</sub> saturates made by reacting C<sub>4</sub> olefins with isobutane using a HF or H<sub>2</sub>SO<sub>4</sub> catalyst), or blends of different types.

The balance of the whole fuel may be made up of other components such as other saturates, olefins, or the like. The olefins are generally formed by using such procedures as thermal cracking, catalytic cracking and polymerization. Dehydrogenation of paraffins to olefins can supplement the gaseous olefins occurring in the refinery to produce feed material for either polymerization or alkylation processes. The saturated gasoline components comprise paraffins and naphthenes. These saturates are obtained from (1) virgin gasoline

by distillation (straight run gasoline), (2) alkylation processes (alkylates) and (3) isomerization procedures (conversion of normal paraffins to branched chain paraffins of greater octane quality). Saturated gasoline components also occur in so-called natural gasolines. In addition to the foregoing, thermally cracked stocks, catalytically cracked stocks and catalytic reformates contain saturated components.

The classification of gasoline components into aromatics, olefins and saturates is well recognized in the art. Procedures for analyzing gasolines and gasoline components for hydrocarbon composition have long been known and used. Commonly used today is the FIA analytical method involving fluorescent indicator adsorption techniques. These are based on selective adsorption of gasoline components on an activated silica gel column, the components being concentrated by hydrocarbon type in different parts of the column. Special fluorescent dyes are added to the test sample and are also selectively separated with the sample fractions to make the boundaries of the aromatics, olefins and saturates clearly visible under ultraviolet light. Further details concerning this method can be found in "1969 Book of ASTM Standards," January 1969 Edition, under ASTM Test Designation D 1319-66T.

The motor gasolines used in formulating the improved fuels of this invention generally have initial boiling points ranging from about 80° to about 105°F. and final boiling points ranging from about 380° to about 430°F. as measured by the standard ASTM distillation procedure (ASTM D-86). Intermediate gasoline fractions boil away at temperatures within these extremes.

From the standpoint of minimizing atmospheric pollution to the greatest extent possible, it is best to keep the olefin content of the fuel as low as can be economically achieved as olefins reportedly give rise to smog-forming emissions, especially from improperly adjusted vehicular engines. Accordingly, in the preferred base stocks of this invention the olefin content will not exceed about 10 volume percent and the most particularly preferred fuels will not contain more than about 5 percent olefins. Table I illustrates the hydrocarbon type makeup of a number of particularly preferred fuels for use in this invention.

TABLE I

| Fuel | Hydrocarbon Blends of Particularly Preferred Base Fuels |         |           |
|------|---------------------------------------------------------|---------|-----------|
|      | Aromatics                                               | Olefins | Saturates |
| A    | 35.0                                                    | 2.0     | 63.0      |
| B    | 40.0                                                    | 1.5     | 58.5      |
| C    | 20.0                                                    | 2.5     | 77.5      |
| D    | 33.5                                                    | 1.0     | 65.5      |
| E    | 36.5                                                    | 2.5     | 61.0      |
| F    | 43.5                                                    | 1.5     | 55.0      |
| G    | 49.5                                                    | 2.5     | 48.0      |

It is also desirable to utilize base fuels having a low sulfur content as the oxides of sulfur tend to contribute an irritating and choking character to smog and other forms of atmospheric pollution. Therefore, to the extent it is economically feasible, the fuel will contain not more than about 0.1 weight percent of sulfur in the form of conventional sulfur-containing impurities. Fuels in which the sulfur content is no more than about 0.02 weight percent are especially preferred for use in this invention.

Normally the gasoline to which this invention is applied is lead-free or substantially lead-free, although small amounts of organolead additives usually employed to give fuels of improved performance quality such as tetraalkyllead antiknocks including tetramethyllead, tetraethyllead, physical or redistributed mixtures of tetramethyllead and tetraethyllead, and the like may be present therein. The gasoline may also contain antiknock quantities of other agents such as cyclopentadienyl nickel nitrosyl, N-methyl aniline, and the like. Antiknock promoters such as tert-butyl acetate may be included. The gasoline may further contain blending agents or supplements such as methanol, isopropanol, t-butanol and the like. Antioxidants such as 2,6-di-tert-butylphenol, 2,6-di-tert-butyl-p-cresol, phenylenediamines such as N,N'-di-sec-butyl-p-phenylenediamine, N-isopropylphenylenediamine, and the like, may be present. Likewise, the gasoline can contain dyes, metal deactivators, or other types of additives recognized to serve some useful purpose in improving the gasoline quality.

Cyclopentadienyl manganese tricarbonyls are known antiknocks and their preparation and use are described in U.S. Pat. Nos. 2,818,417, 2,839,552, and 3,127,351. An important antiknock of this type is methylcyclopentadienyl manganese tricarbonyl. The amount of the cyclopentadienyl manganese tricarbonyl added to the gasoline should be an amount adequate to increase its antiknock effectiveness. This has generally been found to be in the range of from about 0.005 to 10 grams per gallon of manganese as a cyclopentadienyl manganese tricarbonyl. A preferred range is from about 0.05 to 6 gm (grams) of manganese per gallon as a cyclopentadienyl manganese tricarbonyl. A more preferred range is from about 0.05 to about 0.25 gram of manganese per gallon, and a most preferred range is from about 0.05 to about 0.125 gram of manganese per gallon as methylcyclopentadienyl manganese tricarbonyl.

The exhaust gas purification apparatus are well known and generally employ an oxidation catalytic metal such as platinum, rhodium, palladium, or iridium or combinations thereof. Some examples of catalytic converter units are described in U.S. Pat. Nos. 3,441,381 and 3,692,497. The essential elements of such units consist of a catalytic reactor formed by an enlarged cylindrical-frustoconical housing having an inlet port and an outlet port. Located within the housing is a catalyst bed which is a honeycomb alumina-magnesia-silica monolithic ceramic-supported platinum catalyst.

In order to obtain rapid warmup required for catalyst activation, the catalytic reactor is preferably located proximate to the engine exhaust outlet. By proximate is meant that it is close enough that the catalyst bed is rapidly heated to "light off" or activation temperature. The exhaust gas temperature required to accomplish this is dependent upon the nature of the catalyst. Noble metal catalysts containing at least some noble metal such as platinum, palladium or mixtures thereof, activate at lower exhaust temperatures, e.g., 350°-500°F. However, in order to ensure activation, the catalytic reactor is preferably located such that the inlet exhaust temperature is above about 1,000°F. and more preferably above about 1,400°F. during normal engine cruise conditions. It is also at temperatures above about 1,400°F. that the cyclopentadienyl manganese antiknocks are most likely to plug the catalyst and, hence, it is under these conditions that the present invention is

most useful. At temperatures under 1,400°F. plugging of the catalyst does not occur.

In tests run with the aforementioned catalytic converters containing monolithic ceramic supports it has been found that plugging occurs by "spikes" forming on the entrance surface of the cordierite ceramic. These form a network which essentially traps large manganese particles and caps the entrance to the monolithic core.

As stated above, the exhaust gas catalyst unit uses a honeycomb, monolithic ceramic, supported platinum catalyst. These are made by coating a corrugated ceramic structure with an activated alumina and a palladium compound. The preferred ceramics are made using alumina-silica, magnesia-alumina-silica (e.g., cordierite) or mixtures thereof. Palladium can be used in place of platinum, and since these elements generally occur in nature together, it is sometimes preferred to use mixtures of platinum and palladium.

The utility of the invention in alleviating plugging with noble metal catalysts suggests its use with other catalysts if an undesirable amount of plugging is noted. Many non-noble metals have been suggested for exhaust gas catalysts. Examples of other catalytic metals include V, Cr, Mn, Fe, Co, Ni, Cu, Zn, Zr, Na, Mo, Ru, Rh, Ag, W, Re, Os, Ir, Pb, Ba, and the like. These are generally used in an oxide form. They may be used individually or in various groupings such as Cu-Cr, Cu-Cr-V, Cu-Pd, Mn-Cr and the like. They may be supported on the above monolithic ceramic support or on any other of numerous well-known catalyst supports such as granular, pelletized, or extruded alumina, silica, silica-alumina, zirconia, magnesia, alumina-magnesia and the like.

The antiplugging agents of the present invention have the general formula



wherein R is independently selected from hydrogen and hydrocarbyl radicals of preferably up to about 50 carbon atoms and R<sub>1</sub> is independently selected from hydrogen and the



group wherein R' may be hydrogen or a hydrocarbyl radical of up to about 50 carbon atoms. For purposes of this invention a hydrocarbyl radical can be defined as an organic group solely composed of hydrogen and carbon atoms. Some non-limiting representative examples of hydrocarbyl radicals are alkyl, cycloalkyl, aralkyl, alkaryl, and aryl. Preferred hydrocarbyl radicals contain up to about 20 carbon atoms.

Examples of alkyl groups in the above general formula are methyl, ethyl, n-propyl, isopropyl, n-butyl, isobutyl, sec-butyl, tert-butyl, n-amyl, and the various positional isomers thereof, and likewise the corresponding straight and branched chain isomers of hexyl,

heptyl, octyl, nonyl, decyl, undecyl, dodecyl, eicosyl, a polybutene radical of up to 50 carbon atoms, and the like.

When said R, R<sub>1</sub> or R' groups are cycloalkyl groups, they may be cyclopropyl, cyclobutyl, cyclopentyl, cyclohexyl, cycloheptyl, cyclooctyl, cyclononyl, cyclodecyl, cycloundecyl, cyclododecyl, and the like. They may also be such cycloaliphatic groups as α-cyclopropyl-ethyl, α-cyclobutyl-propyl, β-cyclobutylpropyl, and similar alkyl derivatives of the higher cycloalkyls.

When said R, R<sub>1</sub> or R' groups are alkaryl groups, they may be tolyl, 2,3-xylyl, 2,4-xylyl, 2,5-xylyl, 2,6-xylyl, 3,4-xylyl, 3,5-xylyl; o, m, and p-cumaryl, mesityl, o, m, and p-ethylphenyl, 2-methyl-1-naphthyl, 3-methyl-1-naphthyl, 4-methyl-1-naphthyl, 5-methyl-2-naphthyl, 6-methyl-3-naphthyl, 7-methyl-1-naphthyl, 8-methyl-4-naphthyl, 1-ethyl-2-naphthyl, and its various positional isomers and the like.

Examples of aryl groups which may be present in the above general formula are phenyl, naphthyl, and the like.

When said R, R<sub>1</sub> or R' groups are aralkyl groups, they may be benzyl, phenylethyl, 1-phenylpropyl, 2-phenylpropyl, 3-phenylpropyl, 1- and 2-isomers of phenylisopropyl, 1-, 2-, and 3-isomers of phenylbutyl, and the like.

The glycerides, such as the monoglycerides, diglycerides, and specifically the triglycerides having formula I, wherein R is independently selected from hydrogen and hydrocarbyl and R<sub>1</sub> is the



group with R' being independently selected from hydrogen or hydrocarbyl radicals of up to about 50 carbon atoms, are known compounds whose preparation is well known in the art. The chemistry and synthesis of glycerides in general and the triglycerides in particular is adequately treated in Gunston, F. D., *An Introduction To The Chemistry And Biochemistry Of Fatty Acids And Their Glycerides*, Chapman and Hall, Ltd., 1967, particularly in Chapters 5 and 6.

Some non-limiting examples of triglycerides having formula I are glyceryl-3-propionate-1,2-diacetate, glyceryl-2-acetate-1,3-dipropionate, glyceryl triformate, glyceryl triacetate, glyceryl tripropionate, glyceryl tributyrate, glyceryl trivalerate, glyceryl caproate, glyceryl tribenzoate, and the like. Some examples of mono- and diglycerides are glyceryl 1-acetate, glyceryl 2-propionate, glyceryl 1-laurate, glyceryl 1,3-distearate, glyceryl 1-acetate, 3-stearate, and the like. It is

understood that the R and R<sub>1</sub> groups can be the same; two R<sub>1</sub> groups can be the same, while the R group is different; or the two R<sub>1</sub> groups and the R group can all be different. Thus, the R group and the two R<sub>1</sub> groups can be the same alkyl group, the two R<sub>1</sub> groups can be the same alkyl group while the R may be a different alkyl group, or the two R<sub>1</sub> groups and the R group may be different alkyl groups. Likewise, one R<sub>1</sub> may be hydrogen, one R<sub>1</sub> an alkyl group, and the R an aryl group.

The main limitation on the nature of the R, R<sub>1</sub> and R' groups is that they do not make the mono-, di-, or triglyceride insoluble in gasoline or reduce the volatility of said mono-, di-, or triglyceride to a point wherein

said glycerides, and preferably the triglycerides, do not volatilize under the conditions existent in the engine.

Tests were run to illustrate the beneficial effects of the products of this invention on reducing exhaust catalyst plugging with manganese. In such tests a single cylinder engine was used. The A/F mixture was held at approximately 16.0:1 maintaining 1.8% oxygen in the exhaust stream. The engine speed was run generally with a wide open throttle with the spark firing at an appropriate crank angle, depending on engine characteristics and exhaust gas temperature required.

Generally an exhaust gas temperature range of from 1,500°F. to 1,700°F. in the catalyst entrance cone was maintained.

The exhaust catalysts used were PTX units manufactured and sold by Engelhard Industries. The particular PTX unit used was the PTX-3 which is composed of a cordierite ceramic core which has a random stacked, 16 cell/inch configuration. The ceramic has 0.2 wt. percent platinum with 0.5 g Pt on the entire core of the PTX-3 unit. This ceramic is 2.625 inches in diameter, 3.8 inches long and is encased in a Monel mesh to take care of thermal expansion differences between the ceramic and steel housing. This is encased in a stainless steel housing 3 inches in outer diameter and 4 inches long. The ceramic is held firmly in place by two retaining rings on the face of the ceramic welded to the steel casing; in addition  $\frac{1}{8}$  inch square strips are welded to the casing to prevent rotation of the core. The inlet and outlet cover of the unit are 1.5 inches long and the sides form a 45° angle. The casings are joined to a pipe which is connected to the exhaust system. A standard unleaded gasoline of the type described above was used with from 0.25 to 1.0 g Mn/gal as methylcyclopentadienyl manganese tricarbonyl. To determine when the PTX-3 unit was plugged the backpressure in the exhaust stream in front of the PTX-3 unit was measured at predetermined intervals, usually every one or two hours, as the test progressed. The initial backpressure readings generally varied from 0.2 to 0.6 psi. When the back pressure reached a value of 2.0 psi the system was considered plugged and the test was terminated.

The following results were obtained in the above tests when glyceryl triacetate and methylcyclopentadienyl manganese tricarbonyl were used in the test fuel.

TABLE II

| Temp.   | Mn conc. | Glyceryl triacetate conc. | Hours to plug |
|---------|----------|---------------------------|---------------|
| 1500°F. | 1g/gal   | 0                         | 45            |
|         | 1g/gal   | 0.2g/gal                  | 85            |

As demonstrated by the data in Table II when triglycerides, of the type described above are blended with gasoline containing cyclopentadienyl manganese antiknocks reduction of catalyst plugging is obtained.

The amount of antiplugging compound, as for example, glyceryl triacetate, sufficient to reduce the plugging of the catalyst is at least to some extent dependent upon the amount of manganese present in the gasoline and on the inlet exhaust temperature. Generally, the greater the concentration of manganese and the higher the temperature the greater the amount of antiplugging compound needed to reduce plugging of the catalyst.

Generally, the lower limit at which the antiplugging compounds of the present invention are effective to

reduce plugging is about 0.01 g/gal. Preferably, the amount of the compound is greater than 0.03 g/gal, and more preferably greater than 0.125 g/gal. There is no real upper limit on the concentration of the antiplugging compound, and, accordingly, the upper limit is restricted by such secondary considerations as economics, etc. However, 1.0 g/gal of the antiplugging compound, such as glyceryl triacetate, is sufficient to reduce plugging of the catalyst when using a gasoline containing 0.2 g/gal of manganese at a temperature of 1,500°F. Thus, since the amount of the antiplugging compound is quite dependent upon the concentration of the manganese, for practical purposes the upper limit is about 10 g/gal.

Useful gasoline compositions are those which contain from about 0.005 to about 10 grams of manganese per gallon as a cyclopentadienyl manganese tricarbonyl wherein said cyclopentadienyl group is a hydrocarbon group containing from 5 to about 17 carbon atoms and an amount sufficient to reduce plugging of an exhaust gas catalyst of a glyceride, preferably a triglyceride, having formula I.

It is convenient to utilize additive fluid mixtures which consist of cyclopentadienyl manganese tricarbonyl antiknock agents and antiplugging agents having the formula I. These additive fluid mixtures are added to low-lead or unleaded gasoline. In other words, part of the present invention are antiknock-antiplugs fluids which comprise cyclopentadienyl manganese tricarbonyl antiknock agents and the antiplugging agents of the type described hereinabove.

Use of such antiknock-antiplugs fluids in addition to resulting in great convenience in storage, handling, transportation, blending with fuels, and so forth, also are potent concentrates which serve the multipurpose functions of being useful as antiknocks and catalyst plugging reducers.

In these fluid compositions the weight ratio of manganese-to-antiplugging agent can vary from about 0.03 gram of antiplugging agent to 1 gram of manganese or even 0.01 gram of the antiplugging agent to 1 gram of manganese on the one hand to about 10 grams of the antiplugging agent to about 1 gram of manganese on the other hand. Generally, some useful fluids are those that contain 0.03 gram of glyceryl triacetate to 0.125 gram of manganese, 0.06 gram of glyceryl triacetate to 0.125 gram of manganese, 0.2 gram of glyceryl triacetate to 1 gram of manganese, 0.1 gram of glyceryl triacetate to 0.25 gram of manganese, 0.5 gram of glyceryl triacetate to 1 gram of manganese, 1 gram of glyceryl triacetate to 1 gram of manganese, and 2 grams of glyceryl triacetate to 1 gram of manganese. The fluids may optionally contain other additives such as antioxidants, antirust agents, detergents, etc., as well as solvents, e.g., a hydrocarbon, to facilitate handling.

Generally, the amount of the triglyceride present in the additive fluid should be an amount sufficient to reduce plugging of an exhaust gas catalyst when said fluid is added to gasoline. Generally, an additive fluid composition should contain an antiknock amount, i.e., an amount sufficient to reduce knocking, of a cyclopentadienyl manganese tricarbonyl antiknock compound and an antiplugging amount, i.e., an amount sufficient to reduce the plugging of the exhaust gas catalyst, of the glyceride antiplugging compound. An example of an additive fluid composition is one which contains, by weight, 1 part of manganese as cyclopentadienyl manganese tricarbonyl to 2 parts of glyceryl

triacetate.

Although the compounds of the present invention have the most utility when added to gasoline, they can also be used in conjunction with other liquid petroleum distillate fuels such as kerosene, diesel fuel, jet engine fuel, and the like. Claims to the invention follow.

I claim:

1. As a composition of matter, a gasoline for use with an internal combustion engine comprising:
  - i. an antiknock amount of a cyclopentadienyl manganese tricarbonyl antiknock compound wherein said cyclopentadienyl group is a hydrocarbon group containing from 5 to about 17 carbon atoms, and
  - ii. an amount sufficient to reduce the plugging of an exhaust gas catalyst of a glyceride.
2. The composition of claim 1 wherein said cyclopentadienyl group is methylcyclopentadienyl.
3. The composition of claim 2 wherein said glyceride has the general formula



wherein R is selected from hydrogen and hydrocarbyl radicals, and R<sub>1</sub> is independently selected from hydrogen and the

wherein R is selected from hydrogen and hydrocarbyl radicals, and R<sub>1</sub> is independently selected from hydrogen and the



group wherein R' is independently selected from hydrogen and hydrocarbyl radicals.

8. The composition of claim 1 wherein said cyclopentadienyl group is methylcyclopentadienyl.

9. The composition of claim 8 wherein R<sub>1</sub> is a



group.

20 10. The composition of claim 9 wherein R and R' are independently selected from alkyl groups.

11. The composition of claim 10 wherein said alkyl groups are methyl.

25 12. As a composition of matter an additive fluid for low-lead or essentially lead-free gasoline comprising a cyclopentadienyl manganese tricarbonyl antiknock compound, and an amount sufficient to reduce the plugging of an exhaust gas catalyst of a glyceride compound having the general formula

30



35

group wherein R' is independently selected from hydrogen and hydrocarbyl radicals.

4. The composition of claim 3 wherein R<sub>1</sub> is a



40

wherein R is selected from hydrogen and hydrocarbyl radicals and R<sub>1</sub> is independently selected from hydrogen and the



group.

5. The composition of claim 4 wherein R and R' are independently selected from alkyl groups.

6. The composition of claim 5 wherein said alkyl groups are methyl.

7. A substantially lead-free gasoline for use with a noble metal exhaust gas catalyst, said gasoline comprising

- i. an antiknock amount of a cyclopentadienyl manganese tricarbonyl antiknock compound, and
- ii. a glyceride in an amount sufficient to reduce plugging of said noble metal exhaust gas purification catalyst, said glyceride having the general formula



45



group wherein R' is independently selected from hydrogen and hydrocarbyl radicals.

50 13. The composition of claim 12 wherein said cyclopentadienyl group is methylcyclopentadienyl.

14. The composition of claim 13 wherein the R<sub>1</sub> is



group.

15. The composition of claim 14 wherein R and R' are independently selected from alkyl groups.

16. The composition of claim 15 wherein said alkyl group is methyl.

\* \* \* \* \*

65